

Sept. 6, 1932.

H. H. BLAU

1,875,981

INCANDESCENT ELECTRIC LAMP BULB

Filed Sept. 13, 1930



WITNESS  
*AB Wallace.*

INVENTOR

*Henry H. Blau  
By Brown & Critchlow  
Attorneys*

## UNITED STATES PATENT OFFICE

HENRY H. BLAU, OF CHARLEROI, PENNSYLVANIA, ASSIGNOR TO MACBETH-EVANS  
GLASS COMPANY, OF CHARLEROI, PENNSYLVANIA, A CORPORATION OF PENNSYLVANIA

## INCANDESCENT ELECTRIC LAMP BULB

Application filed September 13, 1930. Serial No. 481,618.

The invention relates to incandescent electric lamps having bulbs which are so modified that a substantial portion of the illumination produced by a lamp filament is derived from rays reflected from the modified portion of the bulb, which portion, in addition to functioning as a reflector, is usually translucent to transmit as diffused light a portion of the filament rays which strike it.

10 Illuminating experts have long sought for a durable electric lamp bulb to modify light emanating from a lamp filament in such a way as to combine reduced surface brightness with efficiency in the transmission and reflection of visible radiation, the bulb being relatively free from depreciation both by dis- 15 coloration or deterioration of the material by which it is modified, and being easy and cheap to manufacture.

20 Electric lamp bulbs of the type herein contemplated have been made of clear glass with the bowls of the bulbs provided with enameled portions for increasing their reflecting properties and for diffusing transmitted light. In these kinds of bulbs it has been difficult, if not impossible, to obtain efficiency in illumination and a proper balance between reflected and transmitted light. Also, their manufacture is attended by special operations, such as enameling, which add to the cost of their production, and, in the case of enameled bulbs, the enamel is subject to deterioration. Similarly, some bulbs have had their bowls provided with silver coatings to render them reflecting, and others have been sand blasted or etched to render them translucent. The silvering of such bulbs is objectionable for the reasons stated with reference to the enameling and casing of bulbs, and sand blasted or etched bulbs are inefficient in their light transmitting and reflecting properties. Both sand blasting and enamelling are disadvantageous also because these processes tend to weaken the glass.

25 The object of this invention is to provide an electric lamp bulb which efficiently produces combined direct and indirect illumination, which may be manufactured at a comparatively low cost, and the illuminating effi-

ciency of which will not permanently deteriorate.

The invention is illustrated in the accompanying drawing, of which Fig. 1 is a side view of an electric lamp bulb embodying the 55 invention and shown positioned in a reflector, a cross section of which is illustrated; and Fig. 2 a similar view of a modified form of lamp bulb positioned in an enclosing globe, 60 a cross section of which is illustrated.

It is known to those skilled in this art that the light-transmitting properties of certain glasses may be modified by heat treatment. Specifically, it is known that certain glasses which are normally clear or semi-diffusing 65 may, by heating to a suitable temperature or by retarding their rates of cooling, be rendered diffusing. Glasses of this general type are herein designated as being thermally opacifiable.

70 This invention is predicated upon my discovery that from suitable thermally-opacifiable glass compositions, preferably modifications of those heretofore known to me, an electric lamp bulb may be integrally formed 75 and so thermally opacified locally as to provide it with a translucent portion, which, with low absorption and with low intrinsic brilliancy, transmits from a filament a suitable 80 amount of diffused light, and which portion efficiently reflects a large amount of light through another portion of the bulb which is not thermally opacified. The bulbs thus provided are further characterized by being 85 formed of uniform homogeneous glass, instead of being weakened or modified as is the case in enamelling and sand blasting.

85 In the practice of the invention, a bulb of the desired shape and size for its intended use may be blown in the usual or any desired 90 manner. As is usual, the bulb is preferably formed of substantially uniform thickness throughout. Either as a part of its forming operation, or by a subsequent procedure, the bulb is so treated as to thermally opacify a 95 desired portion of it. When this is done as a part of the forming operation, provision is made for cooling and subsequent reheating of that portion of the bulb which it is desired to thermally opacify, while effecting a 100

normal rate of cooling without such reheating of the glass forming the other portion of the bulb. This may be done by controlling the relative rates of cooling of the parts of a mold adjacent to the two stated portions of the bulb.

When, as is preferred, the thermal opacification of a bulb is effected by a procedure subsequent to the blowing operation, it may be accomplished by heating the portion of the bulb which is to be thermally opacified. This may be done by inserting such portion in a suitable shield or casing electrically or otherwise heated to such a temperature that the portion of the bulb exposed to it is quickly raised to a temperature of from about 950 to 1200° F. The other portion of the bulb should be shielded from the direct action of the heat in such a way that there is produced an adequately sharp line of demarcation between the thermally opacified and un-opacified portions of the bulb. The portion of the bulb desired to be thermally opacified may similarly be inserted in a suitable opening formed in the wall of a gas-fired furnace.

Having reference to the accompanying drawing, an electric lamp is shown in Fig. 1, the lamp including a bulb having its lower portion 2 thermally opacified to transmit diffused light through it and to reflect light through its upper portion 3 for further reflection, by reflector 1, for indirect illumination. The upper portion 3 of the bulb, being untreated, effectively transmits not only the light reflected upwardly from the treated portion 11, but also the direct upward rays from the filament 4 of the lamp. The intrinsic brilliancy of the thermally opacified portion 2 of the bulb being relatively low, the lamp may be viewed without discomfort.

In Fig. 2 an electric lamp having a bulb, such as that just described, is shown positioned within a translucent glass globe 10 such as used for street and like lighting, the bulb of the lamp having its outer or upper portion 11 thermally opacified to transmit diffused light through it and to reflect light downwardly through its untreated lower or socket-end portion 12. The major portion of the light rays from the lamp filament 13 which strikes the treated portion 11 is reflected downwardly through portion 12 and thence through the lower portion of globe 10 for diffused light illumination. Also, direct rays from the filament 13 pass through the lower portion of the bulb for similar illumination. In this way, sufficient light is transmitted through portion 11 of the bulb to illuminate the upper portion of the globe, but without a prejudicial waste of available light.

If desired, a bulb may have one of its sides thermally opacified for use in show cases, in store windows, or in association with shallow reflectors, the combined light transmitting

and reflecting action of the bulb being similar to that just explained. Similarly, the inner portion of a bulb may be thermally opacified for certain particular uses.

The untreated portions of the bulbs are preferably formed of clear transparent glass for the substantially unmodified transmission of both direct and reflected light rays emanating directly and indirectly from the lamp filaments, although in some cases it is desirable to have these untreated portions of the bulbs of a semi-diffusing character to reduce the sharpness of filament images and fixture shadows, as is indicated on the untreated portion 12 of the bulb of Fig. 2. When the untreated portion of a bulb is to be of clear transparent glass, as shown in Fig. 1, the relative proportions of the various constituents of the glass, and particularly the relative proportions of its opacifying to its other constituents, are such that the opacifying constituent or constituents do not exert any opacifying effect under normal heat treatment of the glass. When the untreated portion of a bulb is to be of semi-diffusing character, as shown in Fig. 2, the relative proportions of the various constituents of the glass, and particularly the relative proportions of the opacifying to its other constituents, are such that the opacifying constituent or constituents do not exert their full effect until the bulb is thermally treated in a manner previously explained. With respect to the relative proportions of their opacifying to their other constituents, and the relative proportions of their various constituents to each other, glasses which I have used to obtain the results contemplated by this invention differ from the other thermally-opacifiable glasses known to me.

In the manufacture of bulbs having clear transparent portions for the transmission of reflected and direct light, glasses resulting from the following batches A and B may be used:

| Ingredients                | Batch A   | Batch B   |
|----------------------------|-----------|-----------|
| Sand.....                  | Lbs. 1000 | Lbs. 1000 |
| Soda ash.....              | 290       | 292       |
| Aluminum hydrate.....      | 35        | 38        |
| Feldspar.....              | 680       | 687       |
| Nitre.....                 | 35        | 36        |
| Barium carbonate.....      | 80        |           |
| Arsenic trioxide.....      | 7.5       | 7.7       |
| Sodium silicosilicate..... | 82.5      | 60        |
| Litharge.....              |           | 185       |

In the foregoing batches the constituents are present in such relative proportions and are so balanced with relation to each other that, when melted in a pot heated for about thirty hours at a temperature of about 2625° F. as indicated by an optical pyrometer, there is produced a normally clear transparent glass but one which may be thermally opacified locally to form a dense highly-translucent

glass which is at the same time highly reflecting. In these glasses opacity does not exist unless and until they are thermally treated in a manner previously explained.

5 When the bulbs are formed of a glass which is normally semi-diffusing, they may be made from glasses resulting from the following batches C and D:

| 10 | Ingredients           | Batch C |      | Batch D |      |
|----|-----------------------|---------|------|---------|------|
|    |                       | lbs.    | lbs. | lbs.    | lbs. |
|    | Sand                  | 1000    | 429  | 1000    | 295  |
|    | Soda ash              | —       | —    | —       | 37   |
|    | Aluminum hydrate      | 286     | 738  | 286     | 750  |
|    | Feldspar              | —       | 38   | —       | 37   |
|    | Nitre                 | —       | 71.5 | —       | 36   |
| 15 | Barium sulfate        | —       | 8    | —       | 8    |
|    | Arsenic trioxide      | 286     | 10   | 286     | 83   |
|    | Sodium silicofluoride | —       | —    | —       | —    |
|    | Salt                  | —       | 238  | —       | 192  |
|    | Litharge              | —       | —    | —       | —    |

20 In the glasses resulting from batches C and D the constituents are present in such relative proportions to each other that, when melted in the above-described manner, there is produced a semi-diffusing glass capable of 25 being rendered highly diffusing and highly reflecting by thermal treatment in a manner previously described.

Glasses resulting from the foregoing batches are merely typical, and not limiting. 30 By the use of these and other thermally-opacifiable glasses, bulbs may be thermally opacified locally to form highly diffusing and reflecting portions with adequately sharp lines of demarcation between them and the adjoining glass. Furthermore, the glasses are readily workable, and the thermally opacified portions of bulbs made from them are of uniform opacity.

According to the provisions of the patent 40 statutes, I have explained the principle and operation of my invention, and have disclosed several embodiments of it and examples of how it may be practiced. However, I desire to have it understood that, within the scope 45 of the appended claims, the invention may be practiced otherwise than as specifically illustrated and described.

I claim:

50 1. An incandescent electric lamp bulb integrally formed throughout of a chemically-homogeneous thermally-opacifiable glass, one portion of the bulb being thermally opacified to transmit diffused light and to reflect light through another portion of the bulb.

55 2. An incandescent electric lamp bulb integrally formed throughout of a chemically-homogeneous thermally-opacifiable glass, the bowl of the bulb being thermally-opacified to transmit diffused light and to reflect light through the inner portion of the bulb.

60 3. An incandescent electric lamp bulb integrally formed throughout of a chemically-homogeneous thermally-opacifiable normally clear glass, one portion only of the bulb being thermally-opacified to transmit diffused light

and to reflect light through another portion of the bulb.

4. An incandescent electric lamp bulb integrally formed throughout of a chemically-homogeneous thermally-opacifiable normally semi-diffusing glass, the bowl of the bulb being thermally-opacified to transmit diffused light and to reflect light through the inner semi-diffusing glass portion of the bulb adjacent to its socket end.

75 5. An incandescent electric lamp bulb integrally formed throughout of a chemically-homogeneous glass, one portion of the bulb being differentially opacified throughout its 80 entire body to render it translucent to transmit diffused light and to reflect light through another portion of the bulb.

In testimony whereof, I sign my name.

HENRY H. BLAU.

85

90

95

100

105

110

115

120

125

130